

## UNITED STATES PATENT OFFICE.

JUSTUS W. LEHR, OF BALTIMORE, MARYLAND, ASSIGNOR, BY MESNE ASSIGNMENTS,  
TO U. S. INDUSTRIAL ALCOHOL CO., A CORPORATION OF WEST VIRGINIA.

## NICKEL-COPPER ALLOY.

No Drawing.

Application filed August 28, 1923. Serial No. 659,841.

To all whom it may concern:

Be it known that I, JUSTUS W. LEHR, a citizen of the United States, a resident of Baltimore, State of Maryland, have invented a certain new and useful Nickel-Copper Alloy, of which the following is a specification.

This invention relates to a nickel copper alloy, and more particularly to such an alloy having a comparatively low percentage of nickel and a low percentage of other metals, aside from copper which constitutes the preponderating element in the alloy.

This invention has as an object the provision of a nickel copper alloy which will have a decreased nickel content with respect to Monel metal, but which will not have qualities inferior to Monel metal by reason of such reduction. A further object is to provide a mix for an alloy which will not contain large amounts of soft metals, such as tin or lead, which make the product more fusible but uneven in texture and hardness, and difficult to work. A still further object is to provide a noncorrosive alloy for general use, which will have a high tensile strength and which may be made in the form of white metal at minimum expense, without the high cost due to scrap loss in prior practice. Further objects will appear hereinafter.

The invention in its preferred embodiment consists of an alloy comprising nickel 35 to 40%, tin 2½%, lead 1 to 8%, and the remainder copper; no zinc in any substantial amount is added. A deoxidizer such as silicon, manganese, and zirconium may be used in an amount equal to 1% or less. The nickel percentage may range from 20 to 40%, however, and the percentage of tin may range from 1 to 6%, with corresponding alterations in the percentage of the copper. Such a mix when melted would produce a white metal alloy that has excellent tensile strength and that is eminently suited for making white metal articles that will resist corrosion, such as spigots, pipes, conduits, valves, etc. In making the mix Monel metal is preferably not used since it is desired to

prepare the mix from the pure unalloyed metals and thereby avoid the presence of the small amounts of impurities and other metals naturally present in Monel metal and similar metals.

The metal may be cast by a special process. In casting in a permanent mold, the temperature is controlled to permit a rapid cooling in order to freeze out a maximum concentration of the nickel rich constituent, whereby there will be obtained the advantages of a high nickel alloy while at the same time retaining the total nickel content at a comparatively low figure, so that the difficulties of melting the mix will be lessened. Casting in a permanent iron mold, dusted with graphite, will secure the results desired, and will produce closely joined solid solutions of high nickel and copper content respectively without the formation of inter-crystalline materials.

The alloy produced from the above composition or compositions will possess great strength, uniformity, resistance to corrosion, and a close-grained structure. In these properties, it is equal to and even superior to the well-known Monel metal which has a substantially higher content of nickel.

As many apparently widely different embodiments of this invention may be made without departing from the spirit thereof, it is to be understood that I do not intend to limit myself to the specific embodiment thereof except as indicated in the appended claims.

I claim:

1. A non-corrodible alloy containing nickel 20 to 40%, tin 1 to 6%, lead 1 to 8%, the remainder copper, and containing no zinc.

2. A non-corrodible alloy containing nickel 20% to 40%, tin in a substantial amount not exceeding 6%, lead in a substantial amount not exceeding 8%, and over 45% copper.

3. A non-corrodible alloy containing nickel 20% to 40%, tin in a substantial amount not exceeding 6%, lead in a sub-

stantial amount not exceeding 8%, over 45% of copper, and substantially no zinc.

4. A non-corrodible alloy containing nickel 25 to 45%, tin about 2½%, lead 1 to 8%, and the remainder copper.

5. A non-corrodible alloy containing nickel over 25%, tin about 2½%, lead 1 to 8%, and the remainder copper.

6. A deoxidized non-corrodible alloy con-

taining nickel 25 to 40%, tin 1 to 6%, lead 10 to 8%, and the remainder copper.

7. A deoxidized non-corrodible alloy containing nickel 35 to 40%, tin about 2½%, lead 1 to 8%, and the remainder copper.

In testimony that I claim the foregoing, I have hereunto set my hand this 7th day of August, 1923.

JUSTUS W. LEHR.